

## UNITED STATES PATENT OFFICE

2,323,181

## PRODUCTION OF IMPROVED CELLULOSIC MATERIALS

Richard E. Reeves, Yonkers, N. Y., assignor to  
The Chemical Foundation, Incorporated, a corporation of Delaware

No Drawing. Application May 29, 1939,  
Serial No. 276,442

3 Claims. (Cl. 8—120)

This invention relates to the production of improved textile materials.

The present invention is based upon a selective treatment of cellulosic fibers employed for example in the textile industry.

It has been discovered, as is more particularly explained in the copending application of Wanda K. Farr Ser. No. 270,157, that the cellulose membrane comprises essentially two constituents, crystalline cellulose and an encasing or cementing material having the characteristics of pectous materials. The cellulose material, which occurs in the cellulose membrane, is in the form of ellipsoid particles having the dimensions substantially 1.1 x 1.5 mu. The cellulose particles are remarkably stable and relatively non-reactive and are not, as had previously been supposed, soluble in the typical cuprammonium solutions. In the cell membranes, as for example in cotton fiber, the cellulose particles exist as a definitely oriented phase dispersed in a matrix of the amorphous non-cellulosic (pectous) material. It was found further that many of the characteristics, such as tensile strength, reactivity and the like, which heretofore had been attributed to the cellulose component, were controlled to no inconsiderable degree by the non-cellulosic amorphous material.

The present invention developed from this new conception of the true structure and constituency of the cellulose membrane. Specifically the invention relates to a method of modifying the chemical characteristics of the non-cellulosic constituent associated with cellulose (as for example in cotton fibers) to thereby advantageously modify the physical characteristics of the products produced therefrom.

The broad concept of the invention can best be explained by an illustrative procedure in which the resistance of cellulosic fabric to chemical action is greatly increased, for example an increased resistance to tendering by hypochlorite solutions. The technical value of such an improvement is obvious.

It has been found that the chemical resistance of a cotton fiber or fabric is largely a function of the resistance of the non-cellulosic material. It has been further found that this resistance may greatly be increased by stabilizing the relatively reactive cementitious material by introducing additional grouping therein as for example alkyl and nitro groups.

It is to be observed at this point that the present invention is carefully to be distinguished from earlier suggested methods of modifying the

cellulosic component. For example, while a preferred method of treatment under this invention may be said broadly to be a methylation, in that it involves the use of diazomethane, the purpose and effect of the treatment is entirely different from earlier procedures in which the purpose was to introduce alkyl groups directly into the cellulose molecule. As distinguished from this the present invention relates to the enhancement of the stability of the non-cellulosic material by introducing alkyl or other stability-enhancing groupings therein.

According to a preferred method under the invention the cellulosic material such as cotton thread, woven, knitted or netted cotton fabrics are treated with a solution of diazomethane, controlled as to concentration, temperature and period of contact so as selectively to act upon and modify the non-cellulosic material to thereby improve the chemical and physical characteristics of the fabric. In such preferred method the fabric is contacted in a suitable vessel with an ethereal solution of diazomethane.

In a typical procedure, cotton thread was immersed in a cold solution of 20-30 g. of diazomethane per liter of ether, in the proportion of from 15 cc. to 100 cc. of the solution to 1 gram of the thread. The thread was immersed in the solution for a period of several days. During this period, periodic analysis showed a gradual decrease in concentration of the diazomethane due to the reaction as well as to losses by evaporation and spontaneous decomposition. The material was then removed, washed successively with water, alcohol or ether and air dried.

The product thus produced was chemically analyzed and was found to contain methoxyl groups (5.51%  $\text{OCH}_3$ ). The product was then tested, in comparison with an untreated sample of the same material, to determine the tensile strength before and after treatment with sodium hypochlorite. The results of such tests are shown in the following table:

Table I

|    | Cotton thread                         | Tensile strength             |                                         |
|----|---------------------------------------|------------------------------|-----------------------------------------|
|    |                                       | Before<br>NaOCl<br>treatment | 25 hrs. at<br>25° with<br>N/20<br>NaOCl |
| 50 |                                       | Grams                        | Grams                                   |
|    | Unmethylated.....                     | 1,200                        | 646                                     |
|    | Methylated 5.51% $\text{OCH}_3$ ..... | 1,289                        | 1,092                                   |

It will be observed that the described treatment measurably improves the initial tensile strength of the fabric, in the recorded test about eight per cent. The striking improvement however is in the resistance of the treated material to the deleterious action of the hypochlorite solution. As will be observed after similar treatments in sodium hypochlorite the methylated fabric was almost one hundred per cent stronger than the untreated material. Of equal if not greater significance is the fact that whereas the action of the hypochlorite reduced the strength of untreated cotton to substantially one half the original value, this reagent did not materially reduce the strength of the methylated product, the reduction in strength being only about sixteen per cent.

A most interesting and highly important further effect of this type of treatment is that the treated product shows a very marked resistance to bacterial action, that is to say, to the action of the cellulose-decomposing bacteria. Such a characteristic greatly enhances the value of cotton fabrics which, as is known, are quite susceptible to the action of bacteria and mildew.

As a result of further experimentation, it was determined that the described treatment may readily be employed with all types of cellulosic material to introduce the desired group therein and thus to improve their physical and chemical properties. The following table, in which are recorded the results of treating different types of cellulosic material with the described reagent illustrate their amenability to methylation with the concomitant advantages hereinbefore mentioned.

Table II

| Product treated                                                  | Time | Degree of methylation   |
|------------------------------------------------------------------|------|-------------------------|
| Mercerized cotton.....                                           | Days |                         |
| Raw cotton.....                                                  | 5    | 11.16% OCH <sub>3</sub> |
| Alcohol benzene, H <sub>2</sub> O, 1% NaOH extracted cotton..... | 4    | 5.19% OCH <sub>3</sub>  |
| Spruce wood pulp.....                                            | 5    | 5.48% OCH <sub>3</sub>  |
| Cotton thread.....                                               | 7    | 6.63% OCH <sub>3</sub>  |
|                                                                  | 7    | 5.51% OCH <sub>3</sub>  |

It will be appreciated that it is within the broad concept of the invention to increase the stability of the non-cellulosic material of the cell

membrane by the introduction of a substituent group other than the methyl group, as for example other alkyl groups, nitro groups, and those of a similar character which serve to stabilize the pectous material.

It will be appreciated too that the preferred embodiment herein described presents immediate utility. A treatment of cotton fabrics of the character described increases the resistance and hence the life of such products which during normal use, as in typical laundering, are subjected to the drastic action of hypochlorite or similar bleaching solutions. The invention, therefore not only resides in the broad concept of improving cellulosic products generally, in the respects indicated, but also in the specific improvement of insuring increased longevity of cotton fabrics.

I claim:

1. A method of treating cotton fabrics to impart thereto a marked resistance to the action of hypochlorite solutions which comprises subjecting the fabric to the action of a solution of diazomethane of a concentration of substantially from 20 to 30 grams per liter at below room temperature in the proportion of between about 15 cc. and 100 cc. of solution to about 1 gram of the fabric treated and for a period of several days to effect selective methylation of the pectous non-cellulosic constituent of the fabric.

2. A method of treating cotton fabric to increase their resistance which comprises subjecting the fabric to the action of an ethereal solution of diazomethane of a concentration of about 25 grams per liter in the absence of hydrolyzing agents in the cold for a period of several days to methylate the pectous non-cellulosic constituent of the fibers of the fabric and without any substantial methylation of the cellulosic constituent of the fabric.

3. A method of treating cotton fabrics to impart thereto a marked resistance to the action of hypochlorite solutions which comprises subjecting the fabric in the cold to the action of an ethereal solution of diazomethane of low concentration for a period of several days which will effect selective methylation of the pectous non-cellulosic constituents of the fabric as distinguished from the cellulosic constituents.